

## UNITED STATES PATENT OFFICE

2,370,396

## POWDER METALLURGY

Joseph J. Cordiano, Brooklyn, N. Y., assignor to  
 Hardy Metallurgical Company, New York,  
 N. Y., a corporation of Delaware

No Drawing. Application July 16, 1943,  
 Serial No. 495,031

7 Claims. (Cl. 75—22)

This invention is concerned with powder metallurgy and provides an improved powder for the manufacture of steel objects by compressing and sintering.

It has been proposed heretofore to produce steel objects by compressing and sintering a mixture of relatively pure and soft iron powder with powder of a ferrous alloy containing substantial proportions of combined carbon. The soft iron powder if used in sufficient proportions counteracts the hard and non-coherent nature of the ferrous alloy powder, which by itself does not form strong compacts.

As the result of my investigations, I have developed an improved technique for the manufacture of steel articles by powder metallurgy from a mixture of soft iron powder and a hard ferrous alloy powder such as steel powder, cast iron powder or ferrous alloy powders such as high carbon ferrochrome.

There are a number of important advantages which flow from the practice of my invention including (a) the production of a compact of a higher green strength; (b) a better compact definition, i. e., sharper edges and better molding generally; (c) decreased die wear; (d) increased hardness of the final steel article; (e) an increase in tensile strength of the article; (f) a marked improvement in ductility of the article; and (g) a high resistance to heat shock, so high in fact that excellent permanent molds and dies for casting can be made from the steel powder of my invention.

In accordance with my invention, I employ fine iron powder and fine ferrous alloy powder. Preferably, both powders are all minus 325 mesh. The powders (for example 2 parts of fine soft iron powder and 1 part of fine crushed white cast iron containing, say, 3% of combined carbon) are thoroughly mixed and then heat treated in a non-carburizing atmosphere for a short period, say, 5 to 15 minutes at a temperature (say 700 to 800° C.) sufficient to bring about a fritting together of the fine particles. Thereafter, the fritted agglomerate is subjected to mild comminution, for example by screening on a 100 mesh screen. The screened product is much coarser than the original powders and the majority of the particles in the product consist of sintered agglomerates of fine soft iron particles with fine ferrous alloy particles, the latter containing substantial proportions of combined carbon.

The steel powder produced as described above may be treated in the customary way to form

ferrous objects. The screened powder is compressed in a die of appropriate shape and the resulting green compact is sintered in a protective atmosphere to produce a steel object, which as indicated above will have higher hardness, higher tensile strength and better ductility and resistance to heat shock than an equivalent object made of the same raw materials by exactly the same procedure except that the fritting and screening steps of the invention are omitted.

*Example I*

To take a specific example, 2 parts by weight of a soft iron powder all minus 325 mesh is mixed for 2 hours in a drum type mixer with 1 part of crushed white cast iron powder all minus 325 mesh and containing 3.3% carbon, substantially all of it in a combined state, i. e., as iron carbide. The powder mixture is then heated in a non-carburizing atmosphere, for example an atmosphere of hydrogen, for a time sufficient to bring about a slight fritting together of the particles. Thus the powder mixture may be introduced into a muffle held at 800° C. The introduction of the cold powder mixture will drop the temperature to about 700° C. but in a short time (10 minutes) the temperature will rise to 800° C. The mixture is maintained at this temperature for 5 minutes more and then cooled while it is protected from oxidation.

As indicated above, the atmosphere should be non-carburizing so that the iron powder will not pick up carbon and become hard. An atmosphere of commercial hydrogen is very satisfactory. It is reducing and slightly decarburizing in its action so that any oxides present in the iron powder will be reduced and at the same time there will be a slight decarburization of the cast iron powder, which aids in producing a compressible powder.

The fritted powder is permitted to cool to room temperature in a non-oxidizing atmosphere and is screened through 100 mesh to produce a product of which 25% is minus 100 mesh, 35% is minus 200 mesh and the balance all through 325 mesh. Examination of this powder under the microscope shows that the majority of the particles consist of bonded agglomerates of finer particles of both iron and the ferrous alloy, say white cast iron.

The screened powder may be employed to form steel objects in the customary manner by compressing and sintering. Thus the screened powder may be compressed in a die at 50 tons per square inch to form a green compact which is

removed from the die and sintered for 1 hour at 1200° C. in commercial hydrogen. The sintered compact is then allowed to cool at room temperature and hardened by being heated to 1420° F. in a neutral salt bath and quenched in water.

Steel objects made in accordance with the foregoing procedure have a hardness of 444 Brinell as compared with a hardness of 335 Brinell for an equivalent piece made in exactly the same way except that the powder mixture was not subjected to the preliminary fritting and screening steps to agglomerate the soft iron particles and the cast iron. The procedure is employed to make dies for zinc die castings. The dies are subjected to severe heat shocks but have high durability.

It is not essential to employ powders all of which are minus 325 mesh, since excellent results have been obtained with minus 200 mesh powders.

*Example II*

Approximately 15% of crushed white cast iron powder all minus 325 mesh and containing 3.3% carbon was mixed for 2 hours with approximately 85% of electrolytic iron powder that was substantially free from carbon and all minus 325 mesh.

The mixture was heat treated in an atmosphere of hydrogen at a temperature of 750° C. for a total time of 27 minutes including heating-up time.

The resulting fritted powder mixture was allowed to cool in a non-oxidizing atmosphere to room temperature and then screened through 100 mesh. The screening broke up the larger agglomerates and produced a product of the general nature of that of Example I, except that its combined carbon content was lower, substantially 0.5%.

The screened mixture was compressed in a die at 50 tons per square inch and sintered for 1 hour in hydrogen at 1300° C. The resulting sintered pieces were allowed to cool to room temperature. The cooling was conducted in the furnace. There was no subsequent hardening procedure.

The sintered pieces, after cooling to room temperature, were subjected to tensile testing. They had tensile strengths of 41,300 to 43,600 lbs. per square inch with an elongation in 1 inch of 27%. These values contrast with tensile strengths of 39,200 to 39,900 lbs. per square inch and elongations of 11 to 13% in 1 inch obtained from the same powders in an identical operation, except that the fritting and screening operations were omitted.

As indicated above, the ferrous alloy powder containing the combined carbon need not be white cast iron powder. It may be crushed cast steel powder or for that matter any ferrous alloy containing combined carbon. Thus high carbon ferrosilicon, ferromanganese or ferrochrome powders may be used. Good results may be obtained by employing a small proportion, say 2% of high carbon ferrochrome powder containing 67% chromium and 6% carbon and a larger percentage, say, 14% of crushed white cast iron contain-

ing about 3% carbon, the balance of the mixture being carbon-free iron powder.

If electrolytic iron powder is employed in the practice of the invention, it is desirable to mix the un-annealed electrolytic powder with the ferrous alloy powder and to conduct the fritting operation on this mixture. In this way, the electrolytic iron powder is deoxidized and annealed simultaneously with the fritting operation.

I claim:

1. A steel powder in which the majority of the particles are fritted agglomerates formed by heat treatment of a loose powder mass of finer soft iron particles with finer ferrous alloy particles containing combined carbon.

2. A steel powder in which the majority of the particles are fritted agglomerates formed by heat treatment of a loose powder mass of finer soft electrolytic iron particles with finer cast iron particles containing combined carbon.

3. In the manufacture of steel objects by compressing and sintering a mixture of soft iron powder with harder ferrous alloy powder containing combined carbon, the improvement which comprises subjecting the powder mixture to a preliminary fritting to agglomerate the iron particles and the ferrous alloy particles, and subjecting the resulting fritted mass to mild comminution prior to compressing the powder mixture to form the object.

4. In the manufacture of steel objects by compressing and sintering a mixture of soft iron powder with harder ferrous alloy powder containing combined carbon, the improvement which comprises subjecting the powder mixture to a preliminary fritting to agglomerate the iron particles and the ferrous alloy particles, and subjecting the resulting fritted mass to mild comminution prior to compressing the powder mixture to form the object, the comminution being so conducted that the fritted and comminuted material is substantially coarser than the original powder mixture.

5. A process for producing a steel powder suitable for powder metallurgy which comprises fritting a mixture of fine soft iron particles with fine ferrous alloy particles containing substantial proportions of combined carbon and then subjecting the fritted mixture to mild comminution to produce a powder that is substantially coarser than the original mixture.

6. A process for producing a steel powder suitable for powder metallurgy which comprises fritting a mixture of fine soft iron particles with fine ferrous alloy particles containing substantial proportions of combined carbon at a temperature ranging from 700 to 800° C. and then subjecting the fritted mixture to mild comminution to produce a powder that is substantially coarser than the original mixture.

7. A steel powder in which the majority of the particles are fritted agglomerates formed by heat treatment of a loose powder mass of finer soft iron particles with finer ferrous alloy particles containing iron carbide.

JOSEPH J. CORDIANO.